

## UNITED STATES PATENT OFFICE.

WILHELM UTENDÖRFER, OF COLOGNE, GERMANY.

## PROCESS OF COLORING IRON AND STEEL BLACK.

No Drawing.

Application filed February 15, 1922. Serial No. 536,755.

*To all whom it may concern:*

Be it known that I, WILHELM UTENDÖRFER, a citizen of Germany, and a resident of Cologne, in the Republic of Prussia, Germany, have invented certain new and useful Improvements in Processes of Coloring Iron and Steel Black, of which the following is a specification.

The object of my present invention is to provide a process by means of which articles of iron and steel may be quickly and cheaply colored black. To attain this end I subject said articles to a single working operation in a moderately heated bath of a certain composition, into which bath the articles to be colored are introduced without any preparatory treatment, such as the removal of any fatty matter and the like. On leaving the bath said articles are provided with a permanent black colored coating.

The bath employed for putting my new process into practice consists of dissolved salts resulting from the combination of nitro-phenols with caustic alkalies—as for instance of sodium, potassium, or ammonium—to which solution are added gallic acid and an excess of chemically combined or of free alkali. Very striking results are obtained when the dissolved salts consist substantially of sodium picrate resulting from the combination of trinitro-phenol with caustic soda, to which solution are also added gallic acid and free caustic alkali to such an extent that an excess of free caustic alkali remains. The presence of the gallic acid in said bath causes the formation of a colored coating of an extraordinary deep blue-black.

This bath reaches its full active force, when it has been but moderately heated, for 40 which reason the hardness and the elasticity of any article of iron or steel introduced into said bath does not suffer in any way.

The moderate heating of the bath in combination with the single working operation 45 required by my new process makes it possible that even the most sensitive articles, such as watch springs, precision parts of any description, measuring-instruments, cutting-tools and the like, may be colored black in 60 accordance with my present invention without any detrimental effect.

I claim:

1. The process of coloring iron and steel black consisting in treating the articles to be 55 colored black with a heated solution composed of dissolved salts which result from combining alkali with nitro-phenols, of gallic acid, and of an excess of alkali.

2. The process of coloring iron and steel 60 black consisting in treating the articles to be colored black with a heated solution composed of dissolved salts, which result from combining alkali with nitro-phenols, of gallic acid, and of an excess of free alkali. 65

3. The process of coloring iron and steel black consisting in treating the articles to be colored black with a heated solution composed of sodium picrate, of gallic acid, and of an excess of free caustic alkali. 70

Signed by me at Cologne, Germany, this 21st day of January 1922.

WILHELM UTENDÖRFER.